

Nov. 20, 1951

S. GORDON ET AL

2,575,871

GRANULAR SMOKELESS PROPELLANT POWDERS

Filed Sept. 24, 1947



FIG. 1.



FIG. 2.



FIG. 3.



FIG. 4.



FIG. 5.



FIG. 6.



FIG. 7.

Inventors  
STUART GORDON  
EDWARD WHITWORTH

*Cushman, Harley & Cushman*  
Attorneys

## UNITED STATES PATENT OFFICE

2,575,871

## GRANULAR SMOKELESS PROPELLANT POWDERS

Stuart Gordon, Saltcoats, and Edward Whitworth,  
West Kilbride, Scotland, assignors to Imperial  
Chemical Industries Limited, a corporation of  
Great Britain

Application September 24, 1947, Serial No. 775,950  
In Great Britain December 20, 1946

6 Claims. (Cl. 102—98)

1

The present invention is concerned with improvements in or relating to granular smokeless propellant powders based on colloided nitrocellulose compositions and is particularly concerned with the provision of granular smokeless propellant powders as aforesaid for shot-gun and rimfire cartridges.

It is well known that in the combustion of propellant explosives the amount of gas evolved in any given time for a given composition depends amongst other factors upon the manner in which the burning-surface area varies as burning proceeds. For the aforesaid uses in the case of powders based on colloided nitrocellulose compositions an extremely thin form of grain of large surface area would be necessary which leads to certain difficulties of production. To overcome these difficulties it has long been the practice in the art to incorporate with the ingredients a solid water soluble substance in a fine state of sub-division, and after colloiding the nitrocellulose and forming the powder grains of the preferred size and shape, to leach out the finely divided water soluble ingredient from the powder grains thus leaving a porous structure throughout the propellant grain and consequently large burning-surface, the degree of porosity being controlled by (a) the amount and (b) the grist of the water soluble solid ingredient. It is also well known that porosity improves the ignitability of the grains.

We have now made the discovery that a marked quickening, both as regards ignitability and rate of evolution of gas, can be produced in a porous colloided smokeless propellant composition in disc or flake form by providing it with at least one burning-surface therethrough, as for example, one or more radial slots, or a central perforation with or without one or more radial slots, thereby permitting smokeless propellant powders of at least standard ballistic performance to be produced in the aforesaid manner with less of the finely divided water soluble crystalline ingredients with consequential increased convenience and saving in production.

According to the present invention, therefore, the granular smokeless propellant powders of porous structure based on colloided nitrocellulose compositions, are characterised in that the powders are provided with at least one burning-surface therethrough, as for example, one or more radial slots or a central perforation with or without one or more radial slots.

2

In the drawings, forming part of the specification:

Figure 1 is representative of a granular smokeless perforated disc made in accordance with the invention;

Figure 2 is a radially slotted variation of Figure 1;

Figure 3 is representative of a granular smokeless powder perforated flake;

Figure 4 is a radially slotted variation of Figure 3; and

Figure 5 shows as an example the non-geometric arrangement of the powder granules within a standard type shotgun shell.

15 In the casing 13 of a shotgun shell having the usual head 11 and cap 12, a powder charge 10 made up of the granules having a porous structure 1 and perforations 2 and/or radial slots 3 is randomly packed, above which are placed

20 the usual overpowder card 9, wad 8, undershot card 7, shot 6, overshot card 5, and these are in turn held in place by the turnover 4 of the casing 13.

Figure 6 is representative of a granular smokeless powder flake of this invention having two radial slots therein; and

25 Figure 7 is representative of a granular smokeless powder perforated flake of this invention having one radial slot extending inwardly to said perforation and a second radial slot extending inwardly and stopping short of said perforation.

The following comparative examples illustrate the advantages of the invention.

35 A granular smokeless propellant powder of porous structure is produced in disc form from colloided nitrocellulose (13.25% nitrogen) 100 parts by weight, diphenylamine 1.1 parts by weight, and 65 parts by weight of finely divided 40 potassium nitrate in order to provide the required degree of porosity for a required ballistic performance.

45 Granular smokeless powders of porous structure throughout in disc form and provided in accordance with the invention with a central perforation therethrough give substantially the same ignition and ballistic performance when produced from colloided nitrocellulose (13.25% nitrogen) 100 parts by weight, diphenylamine 1.1 50 parts by weight and potassium nitrate 45-50 parts by weight.

The comparative results are set forth in Table 1.

Table 1

| Sample                                                        | Porosity derived from—                                  | Cartridge                                                 | Gun              | Charge weight, grains | Pressure, tons/m. <sup>2</sup> | Velocity, f. s. |
|---------------------------------------------------------------|---------------------------------------------------------|-----------------------------------------------------------|------------------|-----------------------|--------------------------------|-----------------|
| Powder in square flake form (non-perforated and non-slotted). | 65 pts. potassium nitrate per 100 parts explosive base. | 12 bore 2 3/4" shotgun cartridge with 1 1/4 oz shot load. | 12 bore shotgun. | 32                    | 2.69                           | 1,085           |
| Powder in disc form (non-perforated and non-slotted).         | do                                                      | do                                                        | do               | 32                    | 2.69                           | 1,084           |
| Powder in perforated disc form.                               | 45 pts. potassium nitrate per 100 parts explosive base. | do                                                        | do               | 32                    | 2.67                           | 1,080           |
| Powder in disc form (non-perforated and non-slotted).         | 60 pts. potassium nitrate per 100 parts explosive base. | .410" x 2" shotgun cartridge with 3/8 oz. No. 6 shot.     | .410" shotgun.   | 10                    | 2.63                           | 996             |
| Powder in perforated disc form.                               | 40 pts. potassium nitrate per 100 parts explosive base. | do                                                        | do               | 10                    | 2.94                           | 1,006           |

There is thus a saving of 20%-30% in the amount of potassium nitrate used in the production of granular smokeless propellant powders according to the invention. The formation of sparks is also decreased thereby indicating a more complete combustion of the powder grains.

Comparative results obtained in .22" rifle with standard .22" rimfire ammunition, show improved ignition characteristics for porous powders in perforated or slotted disc form as compared to complete disc form in loose lead and worn rifles denoted by the characteristic small difference between the velocity obtained in a tight lead rifle and the velocity in a worn loose lead rifle. These comparative results are not forth in Table II.

Table II

| Sample                                                          | Charge, wt. grains | Velocity in tight lead rifle | Velocity in worn loose lead rifle | Velocity difference |
|-----------------------------------------------------------------|--------------------|------------------------------|-----------------------------------|---------------------|
| Disc propellant (non-perforated and non-slotted), 30% porosity  | 1.4                | F. s. 1,186                  | F. s. 1,092                       | 94                  |
| Slotted disc propellant, 30% porosity                           | 1.4                | 1,192                        | 1,128                             | 64                  |
| Do                                                              | 1.4                | 1,182                        | 1,124                             | 58                  |
| Disc propellant (non-perforated and non-slotted), 75% porosity  | 1.0                | 1,035                        | 947                               | 88                  |
| Perforated disc propellant, 75% porosity                        | 1.0                | 1,028                        | 981                               | 47                  |
| Disc propellant (non-perforated and non-slotted), 100% porosity | 1.0                | 1,053                        | 974                               | 79                  |
| Perforated disc propellant, 100% porosity                       | 1.0                | 1,052                        | 1,009                             | 53                  |
| Disc propellant (non-perforated and non-slotted), 50% porosity  | 1.0                | 1,046                        | 973                               | 73                  |
| Perforated disc propellant, 50% porosity                        | 1.0                | 1,046                        | 988                               | 58                  |
| Disc propellant (non-perforated and non-slotted), 75% porosity  | 1.0                | 1,010                        | 947                               | 63                  |
| Perforated disc propellant, 60% porosity                        | 1.0                | 1,028                        | 981                               | 47                  |

## We claim:

1. Granular smokeless propellant powders of a porous structure based on colloidal nitrocellulose compositions in the form of powder grains each enclosing in addition to its pores at least one space extending through its entire thickness and defining at least one surface on which the grain may burn outwardly.

2. Granular smokeless propellant powders of a porous structure as set forth in claim 1 wherein said space is a radial slot.

3. Granular smokeless propellant powders of a porous structure as set forth in claim 1 wherein said space is a centrally located perforation.

4. Granular smokeless propellant powders of a porous structure based on colloidal nitrocellulose

compositions in the form of powder grains each enclosing in addition to its pores a plurality of spaces extending through its entire thickness and defining a plurality of surfaces on which the powder grain may burn outwardly.

5. Granular smokeless propellant powders of a porous structure as set forth in claim 4 wherein one of said spaces is a centrally located perforation and the remaining spaces are radial slots.

6. Granular smokeless propellant powders of a porous structure as set forth in claim 4 wherein said plurality of spaces extending through its entire thickness are radial slots.

STUART GORDON.  
EDWARD WHITWORTH.

## REFERENCES CITED

The following references are of record in the file of this patent:

## UNITED STATES PATENTS

| Number    | Name      | Date           |
|-----------|-----------|----------------|
| 677,527   | Maxim     | July 2, 1901   |
| 726,901   | Gathmann  | May 5, 1903    |
| 751,385   | Davis     | Feb. 2, 1904   |
| 802,347   | Aspinwall | Oct. 17, 1905  |
| 899,577   | Wadsworth | Sept. 29, 1908 |
| 1,077,320 | Walsh     | Nov. 4, 1913   |
| 2,261,630 | Regestein | Nov. 4, 1941   |

## FOREIGN PATENTS

| Number | Country       | Date |
|--------|---------------|------|
| 17,994 | Great Britain | 1894 |